

## UNITED STATES PATENT OFFICE.

OTTO MATTHIES AND WALTER DIETERLE, OF DESSAU, AND JOSEF REITSTÖTTER, OF BERLIN-FRIEDENAU, GERMANY, ASSIGNEES, BY MESNE ASSIGNMENTS, TO AGFA ANSCO CORPORATION, OF BINGHAMTON, NEW YORK, A CORPORATION OF NEW YORK.

## PHOTOGRAPHIC SILVER-HALID EMULSION.

No Drawing. Application filed August 6, 1926, Serial No. 127,708, and in Germany September 14, 1925.

- The sensitivity reached in maturing silver halid emulsions depends highly on the gelatine employed. While it is possible with a certain sort of gelatine to attain without any difficulty the desired degree of photographic sensitivity, other gelatines yield only very difficultly or not at all emulsions of a practically useful sensitivity.
- According to the present invention photographic emulsions of high sensitivity may be manufactured by adding in emulsion making products of decomposition of vegetable or animal proteins prepared by alkaline or alkaline fermentative hydrolysis and a simultaneous partial oxidation. These products of hydrolysis, after having been neutralized, can be added directly in the diluted form as they are obtained, or the effective compounds contained therein may first be enriched or isolated. The products of decomposition may be prepared, e. g. from albumin, keratin, gelatine, cystine, animal hide, tendons, cartilages, horn, bone or other raw materials for glue and gelatine.
- It has already been proposed to increase the sensitivity of silver halid emulsions by adding during emulsion making products resulting from a treatment of proteins, but it has been supposed up to now that decomposition in this process would be detrimental to the ability to increase sensitivity and it has always been prescribed to thoroughly avoid any oxidation or bacterial action, i. e., fermentative influence. Thus proteins heretofore have been acted upon for the purpose of producing sensitivity increasing products only in a very mild way. Thus it has been suggested to extract gelatine with distilled water at 30° C. or to extract deliming solutions or powdered pods with organic solvents. We have found that by the decomposition of proteins highly valuable products for the purpose set forth can be obtained. The decomposition may be carried on by hydrolysis, e. g., alkaline hydrolysis, and by initiating oxidation. Such a treatment has been thought to be highly harmful in prior art. It is obvious that the products obtained according to our present invention differ greatly from any prior products intended for the same purpose, since they are breakdown products while heretofore only extracts have been thought applicable. Furthermore, the products extracted by organic solvents are distinguished from our breakdown products by their solubility. Our breakdown products are soluble only in water.
- Since all proteins from animal as well as from vegetable sources may be regarded as aggregates combined of a few fundamental units in varying amounts and in various configurations, the decomposition of any proteins according to the present invention finally yields a solution of nearly the same products, the amount of which only varies with the different sources of material.
- In preparing these products the point at which the decomposition by hydrolysis and partial oxidation is to be stopped, is determined by the refractive index curve of the solution and by testing at regular intervals the photographic qualities of the decomposition products. During the decomposing of proteins the solution shows a continuous increase in the refractive index which tends to reach a constant value when all protein present has been broken down. The photographic test is carried out by making a small batch of emulsion with addition of varying amounts of the product to be tested. From the sensitogram of the resulting emulsion the photographic qualities of the product are easily judged. The decomposing treatment is interrupted when a photographic optimum is reached. In the same way the quantity necessary for any emulsion may be determined.
- By the addition of these products during emulsion making, to the constituents of the emulsion or only to the finished emulsion, one succeeds in obtaining high speed emulsions, though employing a photographically unsensitive gelatine.

## Examples.

1. 10 g. of horn-shavings are boiled with 50 ccm. of a 10 per cent solution of sodium hydroxide, during a rather long time, with supply of air. The filtered and neutralized solution is added during emulsion making or to one of the constituents of the emulsion, when an emulsion is manufactured with 5 kg. of gelatine and 2 kg. of silver nitrate. The sensitivity of the emulsion increases by this treatment from 12° to 17° Scheiner.
2. The same increase of sensitivity is reached by heating for some time 300 g. of

gelatine or 100 g. of calf stock in alkaline solution and adding the neutralized solution during emulsion making or to the gelatine as described in Example 1.

5 3. 100 g. gelatine are hydrolyzed at 37° C. during some hours by pancreatin while keeping the pH-value of the solution at 8 approximately, and the resulting solution is added during emulsion making or to one of the constituents of the emulsion as described in Example 1.

Having now particularly described and ascertained the nature of our said invention and in what manner it is to be performed we declare that what we claim is:

15 1. In the manufacture of photographic silver halid emulsions, the addition to the emulsion of a sensitivity increasing material prepared by alkaline hydrolysis and simultaneous partial oxidation of proteins.

20 2. In the manufacture of photographic silver halid emulsions, the addition to the constituents of the emulsion of a sensitivity increasing material prepared by alkaline hydrolysis and simultaneous partial oxidation of proteins.

25 3. In the manufacture of photographic silver halid emulsions, the addition to the emul-

sion of a sensitivity increasing material prepared by alkaline fermentative hydrolysis and simultaneous partial oxidation of proteins.

4. In the manufacture of photographic silver halid emulsions, the addition to the constituents of the emulsion of a sensitivity increasing material prepared by alkaline fermentative hydrolysis and simultaneous partial oxidation of proteins.

5. Silver halid emulsions having added thereto sensitivity increasing material prepared by the alkaline hydrolysis and simultaneous partial oxidation of proteins.

6. Silver halid emulsions having added thereto sensitivity increasing material prepared by the alkaline fermentative hydrolysis and simultaneous partial oxidation of proteins.

7. Photographic layers comprising the silver halid emulsions of claim 5.

8. Photographic layers comprising the silver halid emulsions of claim 6.

In testimony whereof we affix our signatures.

JOSEF REITSTÖTTER.

OTTO MATTHIES.

WALTER DIETERLE.